

# UNITED STATES PATENT OFFICE.

ALBERT LEIGHTON CROMLISH, OF SHARON, PENNSYLVANIA.

## MANUFACTURE OF SPIEGEL.

1,261,907.

Specification of Letters Patent.

Patented Apr. 9, 1918.

No Drawing.

Application filed January 27, 1917. Serial No. 144,902.

*To all whom it may concern:*

Be it known that I, ALBERT L. CROMLISH, a citizen of the United States, residing at Sharon, in the county of Mercer and State 5 of Pennsylvania, have invented certain new and useful Improvements in the Manufacture of Spiegel, of which the following is a specification.

My invention relates to the manufacture 10 of spiegel, and to the recovery in the form of spiegel of the manganese in "flush" cinder, a hitherto waste product produced in making open hearth steel.

"Flush" cinder and "tapping" cinder are 15 waste products formed in making open hearth steel and produced in large quantities, the flush cinder being obtained when using the well-known pig and ore processes of which the Monell process is one. The 20 flush cinder and also the tapping cinder contains large amounts of manganese as oxids of manganese.

An average analysis of flush cinder will be:

|                      | Per cent. |
|----------------------|-----------|
| 25 Manganese         | 10.25     |
| Iron (by difference) | 37.88     |
| Phosphorus           | .77       |
| Silica               | 22.50     |
| Alumina              | 3.30      |
| 30 Lime              | 17.75     |
| Magnesia             | 7.45      |
| Sulfur               | .10       |

The analysis of flush cinder will vary between the following proportions:

|                      | Per cent.      |
|----------------------|----------------|
| Manganese            | 5.50 to 15.00  |
| Iron (by difference) | 15.00 to 35.00 |
| Phosphorus           | .30 to 2.50    |
| 40 Silica            | 16.00 to 30.00 |
| Alumina              | 2.50 to 5.75   |
| Lime                 | 9.50 to 35.00  |
| Magnesia             | 5.50 to 17.50  |
| Sulfur               | .08 to .12     |

45 The tapping cinder used in forming the burden will have a composition averaging about as follows:

|            | Per cent. |
|------------|-----------|
| Silica     | 36.67     |
| 50 Alumina | 7.43      |
| Lime       | 33.39     |
| Magnesia   | 16.01     |
| Manganese  | 5.00      |
| Sulfur     | 1.50      |

55 One object of the invention is the production of a low manganese spiegel that is

adapted for many uses and particularly in making special steels, as, for example, a steel intended for rolling into sheets, black plate, and tin plate.

60

Another object of the invention is to utilize the "flush" cinder and "tapping" cinder from open hearth furnaces in making low manganese spiegel.

In the manufacture of sheets and tin plate 65 the sheets or tin bars are first rolled in pairs, and the rolled pairs after being matched and doubled are again rolled in packs of "fours" (i. e., four thicknesses of metal). In making light gage materials the packs of "fours" are 70 again doubled and rolled in packs of "eights", and in rolling the light gages the liability of sticking increases.

When steel of the usual composition, which contains not over .04 per cent. phosphorus, 75 is rolled into sheets and tin plate it is found that the sheets or plates will "stick" in the successive rolling operations and cause loss of time, and damage to the rolled materials, in trying to separate the sheets or plates 80 after the rolling operations.

To prevent and overcome the tendency of the sheets and plates to stick when rolled in packs, it has been the practice to slightly increase the phosphorus content of the steel 85 above .04 per cent., (.04 per cent. being the high limit for phosphorus in ordinary commercial steels), it being known that the increased amount of phosphorus in the steel lessens and practically overcomes "sticking" 90 during the rolling operations. Manganese, of course, is always present to some extent in commercial steels.

When making steel to be later rolled into sheets and tin plates, manganese is added to 95 the molten metal, either in the furnace or the ladle, or both, in the form of ferro-manganese or spiegel, and phosphorus in the form of ferro-phosphorus or high phosphorus pig-iron, apatite, and similar materials having a large phosphorus content, also added to the steel to increase its phosphorus content to the desired amount.

Ferro-manganese and spiegel are expensive alloys and ferro-phosphorus or high 10 phosphorus pig iron, apatite, and similar phosphorus bearing materials also are expensive, and at times difficult to obtain.

In practising my invention the "flush" cinder is smelted or reduced in the blast furnace. The burden is reduced in the same 11 manner as when manganese ores are em-

ployed in making ferro-manganese and spiegel, the furnace being tapped at stated intervals and the molten spiegel being cast into pigs in the usual known manner, or when 5 desired being used in a molten condition.

The flush cinder being practically self-fluxing, it is only necessary to add sufficient material to flux the coke charged into the furnace, and when available in sufficient 10 quantities, "tapping" cinder from open hearth furnaces preferably is the flux used.

The necessary amounts of "flush" cinder, which forms the material in the furnace burden from which the manganese in the 15 spiegel is derived, are charged into the blast furnace from time to time, with the required quantities of coke and amounts of fluxing material. When "tapping" cinder is the flux used the entire furnace burden will be formed 20 of "flush" cinder, "tapping" cinder, and coke.

In some cases, as when sufficient quantities of "tapping" cinder are not available, eastern dolomite or similar flux will be substituted for the tapping cinder, or a mixture 25 of part tapping cinder and part dolomite may be used.

Approximately 85 per cent. of the manganese in the "flush" cinder and tapping cinder will be recovered as spiegel.

30 In forming the furnace burden the amount of the various materials charged into the furnace, in pounds per ton of spiegel, will be about as follows:

|                 | Pounds. |
|-----------------|---------|
| 35 Flush cinder | 2839    |
| Tapping cinder  | 5273    |
| Coke            | 3326    |

About 5400 pounds of slag will be formed for each ton of product.

40 When eastern dolomite is used as the flux, the amount in pounds per ton of product of the various materials charged into the furnace in forming the burden will be:

|                 | Pounds. |
|-----------------|---------|
| 45 Flush cinder | 2839    |
| Coke            | 3081    |

Dolomite

With such burden about 4800 pounds of slag will be formed for each ton of spiegel produced.

The resulting product is a low manganese spiegel, a typical analysis of which is

|                      | Per cent. |
|----------------------|-----------|
| Iron (by difference) | 77.18     |
| 55 Manganese         | 13.80     |
| Carbon               | 5.00      |
| Phosphorus           | 3.00      |
| Silicon              | 1.00      |
| Sulfur               | .02       |

When using nothing but cinder in the 60 furnace burden the composition of the spiegel made will vary within the following proportions:

|            | Per cent.      |
|------------|----------------|
| Iron       | 25.00 to 65.00 |
| Manganese  | 13.00 to 25.00 |
| Carbon     | 4.50 to 6.00   |
| Phosphorus | 2.20 to 3.40   |
| Silicon    | up to 1.00     |
| Sulfur     | up to .02      |

70

The utility of my invention will be clearly apparent to those skilled in the art. The manganese in flush and tapping cinder, two hitherto waste products, is reclaimed, and a low manganese, high phosphorus spiegel 75 forming an alloy which is peculiarly adapted for use in the manufacture of steel in making sheets and tin plate, is obtained. The production of a spiegel of the composition claimed provides a cheap substitute for ferro-manganese or spiegel, and ferro-phosphorus or high phosphorus pig iron, and similar expensive materials heretofore necessary in making sheet and tin bar.

80

Modifications in the composition of the materials used to form the furnace burden may be made without departing from my invention. Fluxes other than "tapping" cinder and eastern dolomite may be employed and other changes may be made without departing from my invention as defined in the appended claims.

85

I claim:

1. The process of recovering manganese 95 from flush cinder which consists in charging the flush cinder, coke and tapping cinder into a blast furnace and reducing the so-formed furnace burden, and tapping the furnace to withdraw the molten metal, and thereby forming a low manganese high phosphorus spiegel.

10

2. The process of recovering manganese from flush cinder which consists in charging flush cinder, coke and a flux into a blast furnace, reducing the so-formed burden in the furnace, and tapping the furnace to withdraw the resulting alloy, and thereby forming a low manganese high phosphorus spiegel.

11

In testimony whereof I have hereunto set my hand.

ALBERT LEIGHTON CROMLISH.